

## UNITED STATES PATENT OFFICE

2,055,799

## MANUFACTURE OF SIZED PAPERS

Charles R. Outterson, Watertown, N. Y., assignor  
to Bennett, Incorporated, East Cambridge,  
Mass., a corporation of Massachusetts

No Drawing. Application December 30, 1933,  
Serial No. 704,752

3 Claims. (Cl. 92—21)

This invention relates to the manufacture of sized papers by a process according to which aqueous sizing compositions consisting essentially of stabilized aqueous dispersions or emulsions of unsaponified water-repellent materials are added to paper-making stock in the beater engine and the materials precipitated on the stock by the use of alum or other suitable precipitant preparatory to delivery of the stock to the paper-making machine. Typical of such compositions are aqueous solutions of rosin soap, wherein a substantial amount of rosin is dispersed in free or unsaponified condition; aqueous dispersions of paraffin or other substantially unsaponifiable wax stabilized by rosin soap and containing, if desired, more or less free rosin dispersed therein; and aqueous dispersions of paraffin wax or other substantially inert hydrocarbon wax or bituminous material stabilized by a soap other than rosin soap, for instance, the saponified portion of Montan wax.

Aqueous dispersions of the foregoing kind can be prepared with their dispersed content of unsaponified water-repellent material in a microscopically fine state of sub-division or dispersion. Such fine particle size is of fundamental importance, as it means that the dispersed water-repellent material can be disseminated with substantial uniformity through the paper-making stock in the beater engine and then fixed on the fibers through the action of a precipitant in such a way as to have practically no tendency to separate out during the paper-making operation. Again, the free or unsaponified condition of the dispersed water-repellent material makes for a higher sizing or water-repelling value in the resulting paper with a given usage of sizing material. Thus the use of aqueous rosin soap or size compositions containing a substantial amount of rosin in free or unsaponified condition dispersed therein leads to a better sized paper and one possessing more "snap" and "rattle" than that realized from the same rosin usage in completely saponified condition.

Unfortunately, however, there are instances when excellent aqueous dispersions of the foregoing kind fall down badly in the sizing of paper-making stock in the beater engine in that no matter how fine is their dispersed particle size, the finely dispersed particles agglomerate into coarse ones or the dispersion as a whole coagulates immediately upon addition to the water-slashed paper-making stock, with the result that not only does the resulting paper made from the stock fall far below its expected siz-

ing or water-repelling value, but worse than this, coarse particles of water-repellent material are shed onto and accumulate on the various parts of the paper-making machine, including the web-forming wire cloth, the suction boxes and suction rolls, the transfer felt and the press rolls, and even the drier felt, drier drums, and the calender rolls. In fact, this latter problem may be so serious as to necessitate a stoppage of the paper-making machine and a cleaning of some of its parts at as short intervals as every hour.

There are various instances when a stabilized aqueous dispersion of unsaponified water-repellent material may undergo coagulation or undesirable flocculation upon being added to paper-making stock in the beater engine and hence give rise to the foregoing troubles, but in all instances, the underlying cause is the presence in the beater water, that is, the water serving as the slushing medium for the stock, of electrolytes in sufficient amount to destroy the stabilizer associated with the dispersion and, accordingly, to coagulate or flocculate the dispersed particles before they have been or can be distributed uniformly throughout the stock. Thus, bleached pulps may give trouble when they are not or cannot in practice be washed completely free of bleach or the reaction products of the bleaching operation, as the calcium salts or other chemical residues from the bleaching operation are destructive of the stabilizing agent in the dispersion. The same is true of residual acid, calcium bisulphite, or other calcium salts that may be associated with commercial unbleached sulphite pulps. So, too, difficulty may come from the use of hard waters containing calcium or magnesium salts in slushing the stock in the beater engine or from a similar use of white water recovered from the paper-making machine and containing coagulant, filler, pigment, etc. In fact, two or more of the foregoing undesirable conditions may prevail at once.

In accordance with the present invention, I saponify the water associated with the paper-making stock in the beater engine with substantially completely saponified rosin to such an extent that, although the water may initially have been so charged with electrolyte as to have coagulated an aqueous dispersion of unsaponified water-repellent material, it is rendered practically innocuous toward such dispersion, whereupon such dispersion is uniformly disseminated throughout the stock and the fine particles of water-repellent material are fixed on the fibers by alum or other suitable precipitant. The use

of substantially completely saponified rosin, that is, sodium resinate, for this purpose is distinctly advantageous in that first, it is highly effective in removing from the sphere of potential reaction 5 and precipitating as calcium resinate the calcium ion, which is in many cases the source of trouble, without yielding other troublesome electrolytes as may be true when the usual water-softening agents are employed; second, it may be 10 used in excess to ensure the desired peptizing action and then be precipitated by alum or other suitable precipitant as an effective sizing agent; and, third, it is a comparatively inexpensive agent that is likely to be present or that can be prepared 15 without difficulty in a paper mill. I wish to emphasize the necessity of using substantially completely saponified rosin as the peptizing agent, for should a noteworthy amount of dispersed free rosin be added to a troublesome paper-making 20 stock along with rosin soap, it would be coagulated or flocculated and cause a nuisance on the paper-making machine, as already observed. Once the water component of the stock has been appropriately peptized with substantially completely 25 saponified rosin, the stock may be sized to advantage with an aqueous solution of rosin soap containing a substantial amount of rosin in free or unsaponified condition dispersed therein, with an aqueous dispersion of paraffin wax stabilized 30 with rosin soap, or with any of the other stabilized aqueous dispersions or emulsion of unsaponified water-repellent materials hereinbefore mentioned, for instance, a dispersion of paraffin wax or other inert hydrocarbon wax or bituminous 35 material stabilized by the saponified portion of Montan wax.

It is a comparatively easy matter to determine how my invention should be applied to a given paper-making stock which is troublesome when a 40 stabilized aqueous dispersion of unsaponified water-repellent material is added directly thereto. Thus, I take a sample of the water-slashed stock and quantitatively determine how much of the completely saponified rosin is required to peptize 45 the water with reference to the particular stabilized dispersion of water-repellent material that is to be used in sizing the stock. Or I can introduce into the water-slashed stock, say, about 1% of completely saponified rosin, based on the dry 50 weight of the stock, and, after it has been thoroughly mixed with the stock, withdraw a sample of the water from the stock and add thereto a little of the dispersion to be used as a sizing material so as to determine whether the water associated with the stock contains enough of the saponified rosin to have become peptized thereby. If such is not the case, I can add more completely saponified rosin to the water-slashed stock until I arrive at the point where I can safely introduce 55 thereinto the dispersion to be used as a sizing material. The point at which the stock can be safely treated with the dispersion to be used as a sizing material is that at which the water component of the stock does not generate microscopically coarse 60 particles upon treatment with such dispersion.

A typical specific instance when the principles of my invention were applied to good advantage was in the manufacture of high grade wall paper from a beater furnish consisting partly of 70 bleached sulphite pulp and partly of de-inked and bleached old paper stock. The de-inked and bleached old paper stock had a comparatively short fibrous structure which could not in practice be readily washed clean of bleach and hence 75 contained enough residual bleach to exert a de-

cided coagulating effect upon a rosin size of high dispersed free rosin content and upon a stabilized aqueous dispersion of paraffin wax. In such case, I added to the beater furnished with the bleached sulphite pulp and the de-inked and bleached old paper stock about 1% of completely saponified rosin, based on the dry weight of the stock mixture, ran the beater engine to effect a substantially uniform dissemination of the completely saponified rosin throughout the water component 10 of the stock, and then added an aqueous dispersion of paraffin wax in an aqueous rosin soap solution in the amount of about 1% total solids content, based on the dry weight of the stock. The solids content of the dispersion consisted of 15 about 38% of the paraffin wax and about 62% of the rosin, some of the rosin being in a free or unsaponified condition. After the dispersion had been uniformly incorporated throughout the stock by the operation of the engine, alum was added as 20 ordinarily in sufficient amount to fix the dispersed particles to the stock and the stock run off on a paper-making machine. No trouble was encountered on the paper-making machine as a result of the particular sizing materials employed; and 25 the sizing or water-repelling value of the sizing materials was realized to the fullest extent uniformly throughout the finished paper.

Another typical specific instance when the principles of my invention were applied to good 30 advantage was in the manufacture of a rosin-sized wrapping paper from only unbleached sulphite pulp as the paper-making stock. In such case, the use of rosin size of high free rosin content in the usual manner had given rise to considerable trouble. The fact was that because of the presence in the unbleached sulphite pulp of residual acids and other electrolytes, the addition directly to such pulp in the beater engine of a rosin size composition of high free rosin content 35 occasioned the coagulation of the free rosin and the accumulation of rosin on the Fourdrinier wire and the other parts of the Fourdrinier paper-making machine, causing serious difficulty in the operation of the machine and giving rise 40 to an improperly sized paper. The procedure accordant with the present invention in such case was to introduce into the water-slashed, unbleached sulphite pulp in the beater engine about 45 1% of completely saponified rosin, based on the dry weight of the stock, mix the ingredients thoroughly, and then add to the stock about 2% rosin size solids, based on the dry weight of the stock, in the form of an aqueous rosin size composition containing about 45% free rosin, the 50 rest of the rosin being in the form of sodium resinate. After the rosin size was thoroughly commingled with the stock, alum was used as a precipitant as ordinarily to fix the free rosin and the rosin soap to the stock, and the stock run off 55 on a paper-making machine. The resulting paper was thus sized with rosin size, 30% of which was in free condition. It was characterized by high water repellency and good "snap" and "rattle" by virtue of its free rosin content. If it were attempted to introduce all of the sizing materials at once into the stock in the form of an aqueous sizing composition containing 30% free rosin, serious trouble would ensue on account of coagulation of virtually all of the free rosin. On the other hand, if all of the rosin were used in a 60 completely saponified condition, the desired high sizing value and other qualities sought in the paper would not be attained even though paper-making machine difficulties would be obviated.

My invention extends to other situations wherein difficulty is encountered in the sizing of water-slushed paper-making stock on account of the tendency of such stock to destroy the stability of stabilized aqueous dispersions or emulsions of unsaponified water-repellent materials added thereto for sizing purposes, the foregoing examples being illustrative only. When I say that the water component of the water-slushed stock is "peptized" with substantially completely saponified rosin, I mean that whereas the water component may initially be so charged with electrolytes as to flocculate or coagulate stabilized aqueous dispersions of unsaponified water-repellent materials hereinbefore mentioned added for sizing purposes to the stock, no such tendency exists in the stock whose water component has been treated with the completely saponified rosin which may, in fact, be used in excess so as to render the water component a medium that enhances the stability of the added stabilized aqueous dispersions. Such excess of rosin soap may, however, be precipitated as a sizing material along with the dispersion subsequently added to the paper-making stock and thereby enhance the sizing or water-repelling value realized in the paper made from the stock, as already observed.

I claim:—

30 1. A method of making sized paper which com-

prises first adding to the papermaking stock rosin soap in amount sufficient to peptize the water component of the stock, then adding to the stock a rosin-soap-stabilized aqueous dispersion of unsaponified waterproofing material, said unsaponified waterproofing material including free rosin, precipitating the rosin soap and unsaponified waterproofing material, and running the stock off on a papermaking machine.

2. A method of making sized paper which comprises first adding to the papermaking stock rosin soap in amount sufficient to peptize the water component of the stock, then adding to the stock an aqueous rosin sizing composition, a substantial proportion of whose rosin content is free and the rest of whose rosin content is rosin soap, adding alum to precipitate the rosin soap and free rosin, and running the stock off on a papermaking machine.

3. A method of making sized paper which comprises first adding to the papermaking stock rosin soap in amount sufficient to peptize the water component of the stock, then adding to the stock a rosin-soap-stabilized aqueous dispersion of wax and free rosin, adding alum to precipitate the rosin soap, wax, and free rosin, and running the stock off on a papermaking machine.

CHARLES R. CUTTERSON.

30